

# UNITED STATES PATENT OFFICE.

WILLIAM G. COOK, OF BUSHKILL, PENNSYLVANIA.

## COMPOSITION FOR IMPREGNATING BELTS.

1,334,436.

Specification of Letters Patent. Patented Mar. 23, 1920.

No Drawing.

Application filed August 27, 1919. Serial No. 320,251.

*To all whom it may concern:*

Be it known that I, WILLIAM G. COOK, a citizen of the United States, residing at Bushkill, in the county of Pike and State 5 of Pennsylvania, have invented certain new and useful Improvements in Compositions for Impregnating Belts, of which the following is a specification.

This invention relates to compositions for 10 impregnating fabric, and particularly compositions with which a fabric fan belt or other belt may be impregnated.

The general purpose of the invention is to provide a composition which permits a 15 fabric fan belt to be used, and which will cause this fabric belt to resist the action of oil, but have good frictional engagement with the pulleys or band wheels over which it travels to render the fabric belt somewhat 20 elastic, and to increase its wear.

With these objects in view, my improved composition consists of a mixture of linseed oil, gasolene, a drier of any suitable character, and whiting. These materials are heat- 25 ed and thoroughly mixed and then the fabric, either after it is made into a belt or before, is soaked in this composition until it is thoroughly impregnated therewith. Then the fabric is dried.

The particular action of the various ingredients is that the linseed oil toughens 30 the fabric and causes the fabric to be water- proof and oil-proof. The gasolene makes the mixture more penetrating than it other- wise would be. The drier performs the ob- 35 vious function of causing the compound to

dry quickly, and the whiting acts as a filler for the fabric and increases the frictional engagement of the fabric with the fan wheel or pulley over which it is disposed. 40

Preferably, I make the composition with the materials in the following proportions:

|                   |         |    |
|-------------------|---------|----|
| Linseed oil       | 5 gals. | 45 |
| Gasolene          | 4 gals. |    |
| Whiting           | 5 lbs.  |    |
| An ordinary drier | 1 qt.   |    |

I claim:

1. A composition for impregnating fabric 50 belts including the following ingredients in approximately the following proportions:

|             |         |    |
|-------------|---------|----|
| Linseed oil | 5 gals. |    |
| Gasolene    | 4 gals. | 55 |
| Whiting     | 5 lbs.  |    |

2. A composition for impregnating fabric 60 belts consisting of linseed oil 5 gallons, gasolene 4 gallons, whiting 5 pounds, and a drying oil 1 quart.

3. As an article of manufacture, a fabric 65 belt impregnated with a composition consisting of linseed oil 5 gallons, gasolene 4 gallons, whiting 5 pounds, and an oil drier 1 quart.

In testimony whereof I hereunto affix my signature in the presence of two witnesses.

WILLIAM G. COOK.

Witnesses:

R. G. LUM,  
ERVIN TRANSUE.